

Sept. 30, 1958

2,854,361

W. S. FULKERSON  
METHOD OF REMOVING FOREIGN COATINGS  
FROM TINPLATE AND THE LIKE  
Filed Sept. 9, 1955



INVENTOR  
WILLIAM S. FULKERSON  
BY  
*Gardner & Zimmerman*  
ATTORNEYS

2,854,361

METHOD OF REMOVING FOREIGN COATINGS  
FROM TINPLATE AND THE LIKE

William S. Fulkerson, Hayward, Calif., assignor of one-half to Morris Horwitz, Oakland, Calif.

Application September 9, 1955, Serial No. 533,276

12 Claims. (Cl. 134—30)

This invention relates to the treatment of tinplate, and is more particularly directed to a process for removing coatings of enamel, lacquer, lithographic ink and other materials which might be placed on the tinplate sheets during can manufacturing or other operations.

As is well known in the art, tinplate consists of sheet steel provided with a thin coating of tin, the latter serving to protect the steel from corrosion. Probably the widest use of tinplate is for the manufacture of cans, often referred to as "tin" cans. In the manufacture of such cans, large sheets of tinplate are used, an enamel, varnish or lacquer coating may be placed on the surface which will form the inside of the subsequently formed can body, and the other surface may be likewise coated and/or imprinted with ink. The thus coated sheets are then cut into blanks from which the can bodies are formed.

Notwithstanding the use of good coating and printing equipment, as well as careful quality control, in many cases, the original sheets of tinplate, upon inspection, will be found to have displaced or otherwise defective coatings of lacquer or the like, or the printed material will not be properly positioned on the sheets. Heretofore, when this has occurred, the sheets of tinplate have been discarded and sold for salvage. There is a substantial difference between the cost of tinplate sheets and the salvage price on spoiled sheets, and it has been estimated that the losses resulting from this differential in the can making industry alone run into millions of dollars annually.

It is therefore an object of the present invention to provide a method or process for reclaiming the spoiled tinplate sheets, wherein the inks, lacquers, varnishes and the like which were applied to the sheets, may be readily and economically removed therefrom.

Another object of this invention is to provide a method of the character described which, while effectively removing the surface coatings, will have no deleterious or disturbing effects on the tinplate, nor impart any taste or odors thereto.

A further object of the invention is to provide a tinplate reclaiming process as above described which will permit the use of heretofore spoiled tinplate sheets in the same manner and with the same effectiveness as new sheets.

The invention possesses other objects and features of advantage, some of which, with the foregoing will be set forth in the following description of preferred forms of the invention. It is to be understood, however, that variations in the disclosures of said description may be adopted within the scope of the invention as set forth in the claims.

Referring to the drawing, the figure is a diagrammatic representation of the main steps included in the process of my invention.

In broad terms, the process presently to be described comprises the removal of surface coatings of varnish, lacquer, ink and the like from tinplate sheets so as to

permit the recoating of such sheets where the original coating was in any way defective. As above suggested, there are many reasons why the surface coatings might be defective, for example, the coating covering all or a portion of the surface where the body seam is to be made, the coating being irregular or spotty, the lithographic printing being unclear or not properly positioned, etc. Usually, before such defects have been discovered, a large number of full size sheets will already have been coated and/or printed, and therefore there is a great need for some means of reclaiming these relatively expensive sheets for actual use rather than disposing of them for salvage. It will become clear that the process about to be described can be used where the base sheet is not tinplate, but, for example, a plain steel plate. However, in the case of steel plates, the initial cost more closely approximates the salvage value than where tinplate is involved.

With reference to the diagram of the figure, a tinplate sheet 6 is illustrated in step A, with a defective coating 7 of varnish, lacquer, enamel, or other conventionally used surface coating on one or both surfaces thereof. The coating 7 might likewise include a label printed with ink either on the primary coating or directly on the sheet 6. It is this type of defective sheet that is normally relegated to the salvage pile, but which in accordance with the present invention may be reclaimed and reused. The first step in my process is to take the coated sheet and immerse the same in a bath 8 of isopropyl-monoethanolamine which may be contained in a tank 9, as shown in step B. This bath, when maintained at the proper temperature, serves to loosen the coating 7 from the sheet 6, and may actually effect a complete peeling of the coating from the sheet. It is extremely important to control not only the temperature of the bath, but the time of sheet immersion as well. A short immersion period and/or too low a bath temperature will be ineffective in loosening or peeling the coating from the sheet. Conversely, too long an immersion period and/or too high a bath temperature will readily remove the coating, but will result in stains or other disturbances of the tin layer on its base material, and render the tinplate sheet unusable for can manufacture.

The minimum effective temperature for the isopropyl-monoethanolamine bath is 140° F. for removal of certain coatings without injury to the tinplate. By way of example, conventionally used varnish coatings and lithographic inks will be readily loosened or removed by contact with the bath for approximately 4 minutes, with the bath temperature maintained at 140° F. Lacquer coating removal requires an immersion period of approximately 8 minutes with a bath temperature of about 170° F. Also, where the tinplate sheet was manufactured by the hot dip method, I have found that immersion in a 155° F. bath for approximately 12 minutes is effective in eliminating the stains otherwise found on such sheets. The foregoing temperatures and time periods are naturally dependent to some extent on the thickness of the coatings, but represent actual test figures for conventional can coating thicknesses and materials. If the sheet 6 was plain steel rather than tinplate, the bath temperature could be materially increased, thereby requiring a shorter immersion period, without causing any damage to the sheet.

Thus, in step B, the coated sheet is immersed in a bath of isopropyl-monoethanolamine, maintained at a temperature of 140°-170° F. for a period of from 4 to 12 minutes to effect loosening or peeling of the coating 7 from the sheet.

While the above bath is effective in performing its requisite functions, it is also toxic and must be thoroughly and promptly removed from the tinplate before the lat-

ter may be reprocessed. Therefore, in steps C and D, the sheet is washed with water, which may be sprayed on the sheet, or as indicated in the drawing, the sheet is placed in a tank 12 containing water 13. The water is maintained at a temperature of approximately 140° F. during the washing operation for optimum results. Also, during the washing operation, the sheet is brushed so as to completely remove any traces of the coating from the sheet. If desired, and as shown, a second wash tank 14 may be utilized to insure thorough cleansing of the sheet. Obviously, any suitable strainer or filter system could be incorporated in tanks 9, 12 and 14 so that the removed coating may be continuously or periodically removed from the solution 8 or water 13. As such systems are conventional in the art, and constitute no independent part of my invention, no detailed explanation is deemed necessary, and for the same reason, the thermostatic controls for the solution temperatures have not been illustrated.

Following the water bath, the sheet 6 will be completely free of any portions of the coating 7, but will naturally be wet. The wet sheets must be dried so as to remove all traces of water which will stain tinplate. Therefore, instead of attempting to dry the sheets in more conventional manners, I place the same in a solution 16 of pure alcohol contained in a tank 17 to remove the water. The alcohol may be reused by using copper sulfate crystals to remove the water from the alcohol.

After dipping the sheet in the alcohol bath, step E, the sheet may be dried by a blast of warm air or the alcohol merely permitted to evaporate, in any event leaving a dry sheet of tinplate in excellent condition for receiving a new coating of varnish, lacquer or the like.

The foregoing description sets forth the preferred method of reclaiming tinplate, but it is appreciated that changes might be made which would possibly be effective. By way of example, the time of immersion of the coated sheet in bath 8 could be materially reduced by raising the temperature to say 185° F. This would result in staining the tinplate, but for many manufacturing operations, such staining would not render the tinplate unusable.

Also, for reasons of illustration, the chemical bath 8 into which the defective sheets are placed, has been identified only as isopropyl-monoethanolamine, such material having been thoroughly tested for the purposes set forth. However, while no extensive tests have been conducted, preliminary considerations have indicated that the bath, at the temperatures suggested, could be selected from other ones of the disubstituted amines where one substituent is ethanol and the other is an alkyl radical. Preferably, the alkyl radical contains from three to five carbon atoms, such as found in propyl, butyl and amyl respectively, and even more specifically, the branch chain radicals, such as isopropyl, isobutyl and isoamyl are preferred. Thus, in place of the isopropyl-monoethanolamine, the following liquids appear practical for use, although with possibly diminishing effectiveness:

Isobutyl-monoethanolamine  
Isoamyl-monoethanolamine  
Monoalkylethanolamine  
Propyl-monoethanolamine  
Butyl-monoethanolamine  
Amyl-monoethanolamine

What is claimed is:

1. A method of removing coatings of the character described from metal sheets which comprises applying to said coatings a bath of isopropyl-monoethanolamine maintained at a temperature of from 140° F. to 185° F. for from 3 to 12 minutes, washing said sheets with water to remove said bath, and then drying the sheets.
2. A method of reclaiming tinplate by removing lacquer, varnish, inks and like coatings therefrom comprising: immersing said tinplate in a bath of isopropyl-monoethanolamine to effect a loosening of said coating, washing bath liquid from the tinplate, and then drying the tinplate.
3. The method of removing lacquer, varnish, ink and the like coatings from tinplate which comprises the placing of said tinplate in a bath of isopropyl-monoethanolamine, maintaining the temperature of said bath at from 140° F. to 185° F., removing the tinplate from said bath, and then washing any traces of said bath and said coating from the tinplate.
4. A method as set forth in claim 3 in which said tinplate is kept in said bath for a period of from 3 to 12 minutes.
5. A method of removing oleo and phenolic lacquer coatings from tinplate which comprises heating a bath of isopropylmonoethanolamine to a temperature of approximately 160° F., immersing said coated tinplate in said bath for approximately 10 minutes, removing said tinplate from said bath, applying a water bath at a temperature of about 140° F. to said tinplate, and then drying the tinplate.
6. The method set forth in claim 5 further characterized by said drying including the immersion of the tinplate in an alcohol solution to remove the water therefrom.
7. The method of removing varnish coatings and lithographic inks from tinplate comprising heating a bath of isopropylmonoethanolamine to a temperature of approximately 140° F., immersing said tinplate in said bath for approximately 4 minutes, washing said tinplate to remove said bath, and then drying the tinplate.
8. A method of removing stains from hot dip tinplate comprising heating a bath of isopropyl-monoethanolamine to a temperature of approximately 150° F., immersing the tinplate in said bath for approximately 12 minutes, washing the tinplate to remove the bath therefrom, and then drying the tinplate.
9. A method of removing coatings of the character described from tinplate which comprises applying to said coatings a liquid of a disubstituted amine where one substituent is ethanol and the other is an alkyl radical, heating said liquid to a temperature of from about 130° F. to 185° F., and then washing the liquid from the tinplate.
10. A method as set forth in claim 9 in which said alkyl radical is selected from the group consisting of propyl, butyl, amyl, isopropyl, isobutyl, and isoamyl.
11. A method as set forth in claim 9 in which said liquid is a monoalkylethanolamine.
12. A method as set forth in claim 9 in which said coated tinplate is immersed in said heated liquid for a period of from 3 to 12 minutes.

References Cited in the file of this patent

UNITED STATES PATENTS  
65 2,615,825 Heinecke Oct. 28, 1952